

Sept. 5, 1944.

**A. I. CIDONIO**

**2,357,503**

## METHOD OF MAKING WATERPROOF STRANDS

Filed June 16, 1941



INVENTOR  
ANTHONY J. CIDONIO  
BY *Charles J. Evans*

**ATTORNEY**

## UNITED STATES PATENT OFFICE

2,357,503

## METHOD OF MAKING WATERPROOF STRANDS

Anthony I. Cidonio, San Bruno, Calif., assignor to  
Schor Manufacturing Co., San Francisco,  
Calif., a corporation of California

Application June 16, 1941, Serial No. 398,305

6 Claims. (Cl. 117—55)

My invention relates to an article of the type generally known as gut, such as used for fishing leaders.

It is among the objects of my invention to provide an improved method of producing a superior article of the character described, adapted for rapid production at less cost.

Other objects include the provision of a gut-like article having: greater tensile strength under both dry and wet tests; perfect uniformity of elongation; improved transparency; better flexibility at all temperatures; marked water repellent properties; non-fading azure-blue color; and improved life without loss of its desirable characteristics.

The invention possesses other objects and features of advantage, some of which, with the foregoing, will be set forth in the following description of my invention. It is to be understood that I do not limit myself to this disclosure of species of my invention, as I may adopt variant embodiments thereof within the scope of the claims.

Referring to the drawing:

The figure of the drawing is a diagrammatic view of apparatus illustrating my process.

In terms of broad inclusion, my article comprises a body of filaments treated with certain solutions to sensitize the filaments and to impregnate and coat them with an improved binder. The method comprises forming a body of filaments, preferably grouped in a plurality of strands, and treating it with a solution for cleaning out the pores in the filaments. The body or string is then treated with a second solution containing a colloidal material and a plasticizer to impregnate and sensitize the filaments. After exposing the string thus treated to the air, it is treated with a third solution containing an agent for effecting polarization of the colloid particles. Thereafter it is treated in a fourth solution containing an agent for effecting further polarization and fixation. The string is then preferably treated with fifth and sixth solutions similar to the two last mentioned for further cure. Finally the string is twisted and put on a rack to dry.

In greater detail, and referring to the drawing, I start my process with a plurality of strands or threads 11 each composed of a multiplicity of fine filaments doubled to a specific consistency of about 120 to 215 deniers, 180 deniers being preferred. A denier is the consistency of a thread weighing 1 milligram per 9 meters of

length. I preferably use fibroin filaments. Fibroin is the core portion of silk, comprising the digested mulberry leaves, and is prepared in substantially pure form at the silk house by boiling off the impurities in neat's-foot oil. Chemically, fibroin is a carbohydrate having the formula  $C_{15}H_{23}N_5O_6$ . While fibroin is preferred, it is understood that other filaments, particularly carbohydrates of this general character, may be employed. For example, cotton or flax filaments could be used.

The strands 11 are drawn from freely journaled supply rolls 12, and are then directed into parallelism by suitable means including guide pulleys 13 one of which is shown. These parallel strands thus grouped form a body or string 14 which comprises the foundation of my improved article. The number of strands employed may be varied within wide limits, depending upon the strength desired. I use eight strands in making a 10 pound test leader. For purposes of simplicity four strands are shown. During treatment, string 14 is maintained under a tension of about .025 to 1.25 pounds, .125 pound being preferred. It travels at a rate of from about 16 to 25 feet per minute. A speed of 20 feet per minute is found best in most cases.

Treatment of the fibroin string includes subjecting it to a series of six solutions which will be referred to as solution 1, solution 2, etc. These solutions are retained in tanks 15, the first two of which are adjacent and the last four of which are grouped together at some distance from the first two. String 14 is guided over grooved rollers 17 at the tank edges and submerged by emersion rollers 18 mounted on suitable arms so that they may be withdrawn for threading the string and for cleaning purposes. These rollers are all positively driven to advance the string at the desired rate through the solutions.

Solution 1 functions primarily as a cleaning bath to remove impurities from the pores of the fibroin filaments. Under the microscope it is seen that the filaments contain a multiplicity of minute cores which are clogged with impurities not removed by the boiling off treatment at the silk house. The cleaning solution contains a detergent, preferably an alkali metal salt, such as sodium sulphate or sodium chloride. In order to prevent deposit of the salt on the filaments, an acid is added. A fatty acid such as acetic, or a combination thereof such as acetic and formic acids, or a mineral acid such as sulphuric may be used. In the latter case a

spreader such as sodium bisulfate is preferably added. In my preferred solution, a plasticizer such as diethylene glycol or glycerine is included; the first mentioned being preferred because it is less hygroscopic.

Solution 1 prepares the fibroin for further treatment by cleaning the pores so that the filaments may be impregnated with other materials. This solution also initiates the action of modifying or sensitizing the fibroin itself. The plasticizer is particularly active in this respect. The solution is preferably maintained at a temperature of 100° to 130° F., about 115° being preferred. At the rate of travel designated, the string is exposed to the solution for about 3 seconds, but this time is not critical.

The preferred composition of solution 1, in which the percentages are by weight, is as follows:

|                       | Per cent |
|-----------------------|----------|
| Water                 | 89 to 66 |
| Sodium sulphate       | 2 to 7   |
| Acetic acid (glacial) | 5 to 12  |
| Diethylene glycol     | 4 to 15  |

An alternate solution is:

|                       | Per cent |
|-----------------------|----------|
| Water                 | 86 to 72 |
| Sodium sulphate       | 10 to 20 |
| Acetic acid (glacial) | 3 to 5   |
| Formic acid (90%)     | 1 to 3   |

Another alternate solution is:

|                          | Per cent |
|--------------------------|----------|
| Water                    | 83 to 66 |
| Sodium sulphate          | 10 to 20 |
| Sulphuric acid (66° Bé.) | 2 to 4   |
| Sodium bisulphite        | 5 to 10  |

Solution 2 functions primarily to impregnate and coat the filaments of the string. It contains a colloidal material, preferably a protein colloid; and preferably glutinous in character. My first choice is partially refined animal glue, known as gelatin glue. Casein glue may also be employed. Other colloidal materials, such as gum arabic or bassorin (refined gum tragacanth), may be used. Albumen is also preferably incorporated in the solution to add protein content. The fact that albumen is an irreversible colloid is desirable. A plasticizer, preferably diethylene glycol, is further included in the solution.

The preferred composition of solution 2 is:

|                   | Per cent |
|-------------------|----------|
| Water             | 30 to 45 |
| Gelatin glue      | 35 to 50 |
| Albumen           | 20 to 2  |
| Diethylene glycol | 15 to 3  |

An alternate solution is:

|              | Per cent |
|--------------|----------|
| Water        | 20 to 30 |
| Gelatin glue | 20 to 35 |
| Albumen      | 35 to 15 |
| Glycerine    | 25 to 20 |

While I refer to this treating bath as a solution along with the others for the sake of a common term, it is not a true solution but a colloidal dispersion. As the string passes through it the filaments are impregnated and coated with the colloidal material; and, since the microscopic pores were previously cleaned out, the treating material effectively permeates and saturates the individual filaments as well as coating them and the strands as a whole. Here again the solution also functions to modify or sensitize the fibroin itself, due

particularly to the plasticizing agent; diethylene glycol being preferred over glycerine as a plasticizer because it is less hygroscopic. The solution is maintained at a temperature of 80° to 110°

5 F., about 95° being preferred.

From solution 2 the coated string is exposed to the atmosphere for a run of about 30 feet at a room temperature of about 65° to 75° F. with a relative humidity of say 30° to 60°. At the rate 10 of travel indicated this provides an exposure of about 1 minute 30 seconds, although that time is not critical. The strands of the string are then compressed into cylindrical shape and excess coating material is removed by passage through 15 an apertured rotor in a block 19. The rotor aperture is flared at both ends and has a central restricted throat having a diameter about twice the dry size of the leader being made. This rotor puts a partial twist in the string, which tends to 20 compact the strands and form them into a true cylinder, and also scrapes and spins off the excess coating material.

String 14 then passes through solution 3 containing an agent which functions to effect first 25 degree polarization of the colloidal material, causing orientation and condensing or compacting of the ionized colloid particles. Potassium chromium sulphate is the preferred agent. Other salts such as potassium chloride and chromium chloride may be used. The chromium salts are 30 preferred because they react with the formaldehyde later used to give the desired color for a leader.

The preferred composition of solution 3 is:

|                             | Per cent |
|-----------------------------|----------|
| Water                       | 97 to 74 |
| Chromium potassium sulphate | 3 to 26  |

The string then passes through solution 4 containing an agent for effecting further polarization and fixation of the colloid particles. Formaldehyde is the preferred agent because it also reacts with the potassium chromium sulphate to 40 impart a non-fading pigment of azure-blue color ideal for a leader. Potassium dichromate may be used as a fixing agent but the color imparted 45 is not so good for fishing leader purposes.

The preferred composition of solution 4 is:

|              | Per cent |
|--------------|----------|
| Water        | 80 to 98 |
| Formaldehyde | 20 to 2  |

In order to further cure the impregnating and coating material, the string is preferably treated with two additional solutions 5 and 6 similar to those last mentioned.

The preferred composition of solution 5 is:

|                             | Per cent |
|-----------------------------|----------|
| Water                       | 95 to 87 |
| Chromium potassium sulphate | 5 to 13  |

The preferred composition of solution 6 is:

|              | Per cent |
|--------------|----------|
| Water        | 95 to 90 |
| Formaldehyde | 5 to 10  |

From solution 6 the string passes through another apertured rotor in a block 21 which further compresses and forms it and scrapes off excess coating material. Then the end of the 70 string is attached to a carriage 22 having means for twisting the strands. The twisting means is timed with the carriage movement to impart three twists to the inch. After the carriage has traveled out to the end of its path, which may be any suitable distance, say 40 yards, the feed-

ing of the string through the apparatus is stopped and the string is cut adjacent block 21; whereupon the carriage is returned to twist a new length. If desired, a fixed twisting head may be provided in place of the carriage, so that the string is twisted as it passes through the head, thus making the process continuous.

The twisted product is then placed on a rack at room temperature to dry for a period of about 1½ hours. If desired, the leaders may be polished with sand paper and given a sheen with oil.

The gut-like product thus produced is an excellent fishing leader. It is materially stronger under both wet and dry tests than ordinary leaders, and is uniform in strength and elongation throughout its length. It is very flexible under all ordinary temperatures; may be knotted with minimum loss of tensile strength; and is exceedingly water repellent. The product has marked transparency, and possesses a non-fading azure-blue color that is ideal for a fishing leader, making it substantially invisible in the water. Furthermore, the product retains its desirable characteristics over a long period.

While my product is an excellent fishing leader, it is to be understood that it may be used for any purpose where gut-like materials are employed. Strings for playing rackets, and surgical sutures are a few of such uses.

I claim:

1. The method of making an article which comprises forming a body of fibroin filaments cleansed by treatment with a detergent, impregnating the filaments with a protein colloidal material, partially drying the impregnated filaments, treating the body with a solution of a polarizing salt, then treating it with a solution containing a substance in the class consisting of formaldehyde and potassium dichromate, and then repeating the two treatments last mentioned.

2. The method of making an article which comprises forming a body of fibroin filaments, treating the filaments with a detergent in the presence of a plasticizer, impregnating the filaments with a protein colloidal material, partially drying the filaments, treating the body with a solution of a polarizing salt, and then treating it with a solution containing a substance in the class consisting of formaldehyde and potassium dichromate.

3. The method of making an article which comprises forming a body of fibroin filaments cleansed by treatment with a detergent, impregnating the filaments with a colloidal material including albumen and a hardenable organic colloidal material, treating the body with a solution of a polarizing salt, and then treating it with a solution containing a substance in the class con-

sisting of formaldehyde and potassium dichromate.

4. The method of making an article which comprises forming a body of fibroin filaments and then successively treating the body with the following solutions:

Solution 1, containing a detergent

Solution 2, containing a protein colloidal material

10 Solution 3, of a polarizing salt  
Solution 4, containing a substance in the class consisting of formaldehyde and potassium dichromate.

15 5. The method of making an article which comprises forming a body of fibroin filaments, and then successively treating the body with the following solutions containing ingredients in proportions by weight of:

20 *Solution 1*

|                      | Per cent |
|----------------------|----------|
| Water                | 89 to 66 |
| Sodium sulphate      | 2 to 7   |
| Acetic acid          | 5 to 12  |
| 25 Diethylene glycol | 4 to 15  |

25 *Solution 2*

|                   |          |
|-------------------|----------|
| Water             | 30 to 45 |
| Gelatin glue      | 35 to 50 |
| 30 Albumen        | 20 to 2  |
| Diethylene glycol | 15 to 3  |

30 *Solution 3*

|                                |          |
|--------------------------------|----------|
| Water                          | 97 to 74 |
| 35 Chromium potassium sulphate | 3 to 26  |

35 *Solution 4*

|              |          |
|--------------|----------|
| Water        | 80 to 98 |
| Formaldehyde | 20 to 2  |

40 *Solution 5*

|                             |          |
|-----------------------------|----------|
| Water                       | 95 to 87 |
| Chromium potassium sulphate | 5 to 13  |

45 *Solution 6*

|              |          |
|--------------|----------|
| Water        | 95 to 90 |
| Formaldehyde | 5 to 10  |

60 6. The method of making fishing leaders which comprises grouping a plurality of fibroin filaments, treating the filaments with a detergent in the presence of a plasticizer, impregnating the filaments with a protein colloidal material, treating the impregnated filaments with a solution of a polarizing salt for effecting a first degree of polarization of the colloidal material, then treating the filaments with a solution of formaldehyde for effecting further polarization and fixation of the colloidal material, and twisting the treated filaments.

ANTHONY I. CIDONIO.